

D. L. H. FORBES,  
CYANIDE PROCESS OF TREATING ORES OF THE PRECIOUS METALS,  
APPLICATION FILED APR. 3, 1922.  
1,430,635.

Patented Oct. 3, 1922.



INVENTOR,

D. L. H. Forbes,  
J. Edward Maybee.  
ATTY.

Patented Oct. 3, 1922.

1,430,635

# UNITED STATES PATENT OFFICE.

DAVID L. H. FORBES, OF KIRKLAND LAKE, ONTARIO, CANADA.

## CYANIDE PROCESS OF TREATING ORES OF THE PRECIOUS METALS.

Application filed April 3, 1922. Serial No. 549,307.

To all whom it may concern:

Be it known that I, DAVID L. H. FORBES, of Kirkland Lake, in the district of Timiskaming, Province of Ontario, Canada, a subject 5 of the King of Great Britain, have invented certain new and useful Improvements in Cyanide Processes of Treating Ores of the Precious Metals, of which the following is a specification.

10 This invention relates to the treatment of ores of the precious metals, and more particularly ores containing tellurides of the precious metals, by the well known cyanide process.

15 When unroasted ores containing such tellurides are treated according to the most approved modern practice, the loss is often as much as from 15% to 20% of the gold present, whereas with ordinary ores it is possible, 20 economically to recover all but 3% to 4% of the gold. My object therefore is to devise an economically practicable method of increasing the recovery of precious metals from ores containing tellurides. The essentials, chemically, of such a process seem to be the presence in the ore pulp of nascent oxygen, strong caustic, and a minimum of cyanide. A further physical essential is that the nascent oxygen be generated in such a manner 25 that it does not escape from the pulp until it has had full opportunity of coming into intimate contact with the ore particles.

I attain the desired conditions both chemically and physically by injecting powdered 30 sodium peroxide beneath the surface of a mixture of the ground ore and cyanide solution, preferably by means of the action of a blast of compressed air.

Apparatus adapted for this purpose is 35 shown in the accompanying drawing, which is a side elevation of the apparatus, partly broken away.

1 is a tank adapted to contain a mixture of comminuted ore and cyanide solution. 40 Above the tank is suitably supported a receptacle 2 for the powdered sodium peroxide. This is provided with a suitable cover such as a screw cap 3. The lower end of the receptacle is provided with a discharge pipe 4, 45 which extends downwardly to a position well below the normal surface level of the contents of the tank. A compressed air pipe 5 is led from a suitable source of compressed air and opens through the side of the receptacle 2, preferably just above the outlet 50

opening to the pipe 4. A control valve 6 is provided in the pipe 5, the valve stem being provided with an indicator finger 7 movable over a scale 8. The valve may thus be readily set to vary the air pressure to feed 60 any desired quantity of the sodium peroxide, the air entraining the sodium peroxide as it passes from the receptacle. Both the peroxide and air escaping from the lower end of the pipe 4, not only is sodium peroxide thus 65 delivered to a point well below the surface of the material in the tank, but the air, which is used to feed the peroxide, also serves either alone or with the air of any mechanical adjuncts to effect the necessary 70 agitation of the pulp.

A moisture trap 9 of any known type is preferably inserted in the pipe 5 to take moisture out of the air, which otherwise would tend to break up the peroxide before 75 it reached its proper point of application.

In the practical application of my process I follow the usual practice of reducing the ore and grinding it in cyanide solution until the desired degree of fineness is reached, and 80 of treating the ground ore in agitation tanks. My process, however, differs from that commonly employed in that into one or more of the agitation tanks, or at some other convenient stage in the process I inject sodium 85 peroxide by means of the apparatus hereinbefore described or by any other means. From this it results that nascent oxygen liberated by the action of the liquid on the sodium peroxide, as well as the resulting strong 90 caustic soda solution, comes into intimate contact with the fine particles of ore before the oxygen has a chance to escape from the moisture. While I have found that a continuous injection of sodium peroxide at a 95 uniform rate gives the best results, I have also found that intermittent injection is beneficial. In practice I have found that the injection of sodium peroxide in proportions even as small as one-quarter of a pound of 100 sodium peroxide per ton of ore treated gives an increased recovery greater than the cost of the treatment. On average ores one-half of a pound of sodium peroxide per ton may be used to advantage, while, on rich ores, 105 proportions as much as three to five pounds per ton or more may be used to advantage, it being necessary, however, to keep in mind the fact that the upper limit would be set in practice by the percentage of caustic soda 110

that could be carried safely in the solution without interfering with the subsequent settling, filtering or precipitation operations.

A further benefit resulting from my process lies in the changed character of the gold-silver-zinc precipitate that is obtained from the pregnant solution. When treating telluride ores, as above described, I have found that there is a very marked decrease in the proportion of tellurium present in this precipitate and that the volatilization loss of gold when melting the precipitate into bullion bars is correspondingly reduced.

While I am aware that oxidizing reagents have been suggested in the treatment of gold and silver ores by the cyanide process, I am not aware that they have been employed in the treatment of ores containing tellurides of gold and silver, and it has not heretofore been suggested that the most economical results could only be obtained by injecting such reagents, and particularly sodium peroxide, below the surface of the mixture of ore in the cyanide solution and preferably by means of compressed air.

What I claim as my invention is:-

1. The process of treating ores containing precious metals which consists in injecting small quantities of dry sodium peroxide below the surface of a mixture of comminuted ore and cyanide solution.

2. The process of treating ores containing precious metals which consists in injecting small quantities of dry sodium peroxide below the surface of a mixture of comminuted ore and cyanide solution with and by means of compressed air.

3. The process of treating refractory ores

of the precious metals containing tellurides of gold or silver which consists in introducing small quantities of dry sodium peroxide into a mixture of comminuted ore and cyanide solution.

4. The process of treating refractory ores of the precious metals containing tellurides of gold or silver which consists in injecting small quantities of dry sodium peroxide below the surface of a mixture of comminuted ore and cyanide solution.

5. The process of treating ores containing precious metals which consists in injecting small quantities of dry sodium peroxide below the surface of a mixture of comminuted ore and cyanide solution and thoroughly agitating the mixture.

6. The process of treating refractory ores of the precious metals containing tellurides of gold or silver which consists in introducing small quantities of dry sodium peroxide into a mixture of comminuted ore and cyanide solution and thoroughly agitating the mixture.

7. The process of treating refractory ores of the precious metals containing tellurides of gold or silver which consists in injecting small quantities of dry sodium peroxide below the surface of a mixture of comminuted ore and cyanide solution with and by means of compressed air.

Signed at Kirkland Lake this 25th day of March 1922.

DAVID L. H. FORBES.

Witnesses:

M. DE LISLE,  
L. A. LILLICE.